



US011453836B2

(12) **United States Patent**  
**Wendker et al.**

(10) **Patent No.:** **US 11,453,836 B2**  
(45) **Date of Patent:** **Sep. 27, 2022**

(54) **LUBRICANT COMPRISING A LIQUID ETHYLENE COPOLYMER**

(71) Applicant: **BASF SE**, Ludwigshafen am Rhein (DE)

(72) Inventors: **Martin Wendker**, Ludwigshafen am Rhein (DE); **Ivette Garcia Castro**, Ludwigshafen am Rhein (DE); **Jan Strittmatter**, Ludwigshafen am Rhein (DE); **Karolin Geyer**, Ludwigshafen am Rhein (DE); **Wolfgang Grabarse**, Ludwigshafen am Rhein (DE); **Markus Scherer**, Ludwigshafen am Rhein (DE); **Rene Koschabek**, Ludwigshafen am Rhein (DE)

(73) Assignee: **BASF SE**, Ludwigshafen am Rhein (DE)

(\*) Notice: Subject to any disclaimer, the term of this patent is extended or adjusted under 35 U.S.C. 154(b) by 0 days.

(21) Appl. No.: **16/981,569**

(22) PCT Filed: **Mar. 14, 2019**

(86) PCT No.: **PCT/EP2019/056402**

§ 371 (c)(1),

(2) Date: **Sep. 16, 2020**

(87) PCT Pub. No.: **WO2019/175300**

PCT Pub. Date: **Sep. 19, 2019**

(65) **Prior Publication Data**

US 2021/0246395 A1 Aug. 12, 2021

(30) **Foreign Application Priority Data**

Mar. 16, 2018 (EP) ..... 18162296  
Jul. 18, 2018 (EP) ..... 18184185

(51) **Int. Cl.**

**C10M 143/00** (2006.01)  
**C10M 143/02** (2006.01)  
**C10M 145/14** (2006.01)  
**C10M 169/04** (2006.01)  
**C10N 20/00** (2006.01)  
**C10N 20/02** (2006.01)  
**C10N 20/04** (2006.01)  
**C10N 30/02** (2006.01)

(52) **U.S. Cl.**

CPC ..... **C10M 143/02** (2013.01); **C10M 145/14** (2013.01); **C10M 169/041** (2013.01); **C10M 2205/022** (2013.01); **C10M 2209/084** (2013.01); **C10N 2020/011** (2020.05); **C10N 2020/019** (2020.05); **C10N 2020/02** (2013.01); **C10N 2020/04** (2013.01); **C10N 2030/02** (2013.01)

(58) **Field of Classification Search**

CPC ..... C10M 143/02; C10M 145/14; C10M

169/041; C10M 2205/022; C10M 2209/084; C10M 2203/1006; C10M 2203/1025; C10M 2203/1065; C10M 2205/0285; C10M 2207/2805; C10M 2209/1033; C10M 2223/0405; C10M 2229/025; C10M 107/28; C10M 107/04; C10N 2020/011; C10N 2020/019; C10N 2020/02; C10N 2020/04; C10N 2030/02

See application file for complete search history.

| <b>References Cited</b> |         |                                     |
|-------------------------|---------|-------------------------------------|
| U.S. PATENT DOCUMENTS   |         |                                     |
| 3,404,091 A             | 10/1968 | Takashima et al.                    |
| 3,621,004 A *           | 11/1971 | Eckert ..... C08F 210/00<br>526/320 |
| 4,261,703 A             | 4/1981  | Tack et al.                         |
| 2004/0097751 A1         | 5/2004  | Fechtenkotter et al.                |
| 2010/0048439 A1         | 2/2010  | Maelhling et al.                    |
| 2012/0005951 A1         | 1/2012  | Maelhling et al.                    |
| 2017/0335033 A1         | 11/2017 | Voellmar et al.                     |
| 2019/0169346 A1         | 6/2019  | Misske et al.                       |

FOREIGN PATENT DOCUMENTS

|    |                  |         |
|----|------------------|---------|
| CA | 869589 A         | 4/1971  |
| DE | 2921330 A1       | 12/1979 |
| WO | WO-2004106471 A1 | 12/2004 |
| WO | WO-2018024563 A1 | 2/2018  |
| WO | WO-2019175301 A1 | 9/2019  |

OTHER PUBLICATIONS

International Search Report for PCT/EP2019/056402 dated Jul. 11, 2019.

International Search Report for PCT/EP2019/056404 dated Jun. 6, 2019.

Written Opinion of the International Searching Authority for PCT/EP2019/056402 dated Jul. 11, 2019.

Written Opinion of the International Searching Authority for PCT/EP2019/056404 dated Jun. 6, 2019.

Buback, et al., "Development of a High-Pressure High-Temperature Stirred Vessel with Incidence of Light for Continuous Operation", Chemie Ingenieur Technik, vol. 66, Issue 4, Apr. 1994, pp. 510-513.

European Search Report for EP Patent Application No. 18162296.0, dated May 29, 2018, 3 pages.

\* cited by examiner

Primary Examiner — Taiwo Oladapo

(74) Attorney, Agent, or Firm — Faegre Drinker Biddle & Reath LLP

(57) **ABSTRACT**

The present invention relates to a lubricant comprising a liquid ethylene copolymer which comprises in polymerized form 20 to 60 wt % of ethylene; and at least 20 wt % of an acrylate, which is selected from C1-C22 alkyl (meth)acrylate. It further relates to the liquid ethylene copolymer; and to a method for reducing friction between moving surfaces comprising the step of contacting the surfaces with the lubricant or with the ethylene copolymer.

18 Claims, No Drawings

## 1

LUBRICANT COMPRISING A LIQUID  
ETHYLENE COPOLYMERCROSS-REFERENCE TO RELATED  
APPLICATIONS

This application is a national stage application (under 35 U.S.C. § 371) of PCT/EP2019/056402, filed Mar. 14, 2019, which claims benefit of European Application Nos. 18162296.0, filed Mar. 16, 2018, and 18184185.9, filed Jul. 18, 2018, all of which are incorporated herein by reference in their entirety.

The present invention relates to a lubricant comprising a liquid ethylene copolymer which comprises in polymerized form 20 to 60 wt % of ethylene; and at least 20 wt % of an acrylate, which is selected from  $C_1$ - $C_{22}$  alkyl (meth)acrylate. It further relates to the liquid ethylene copolymer; and to a method for reducing friction between moving surfaces comprising the step of contacting the surfaces with the lubricant or with the ethylene copolymer. Combinations of preferred embodiments with other preferred embodiments are within the scope of the present invention.

Object was to find ethylene copolymers for lubricants, which should overcome the drawbacks of the prior art. For example the ethylene copolymers or the lubricant comprising the ethylene copolymers should be liquid, should have a low pour point, a good miscibility with apolar base stocks, a good miscibility with polar base stocks, a good oxidation stability, a high viscosity index, a low friction coefficient, a low volatility, a high chemical stability, a high shear stability, a viscosity index, a low sludge, a high cleanliness, a good thickening efficiency, a high hydrolytic stability, or good cold flow properties. Preferably, the ethylene copolymer or the lubricant comprising the ethylene copolymers should provide a combination of several of such advantages.

The object was solved by a lubricant comprising a liquid ethylene copolymer which comprises in polymerized form 20 to 60 wt % of ethylene; and

at least 20 wt % of an acrylate, which is selected from  $C_1$ - $C_{22}$  alkyl (meth)acrylate.

The object was also solved by the liquid ethylene copolymer; and by a method for reducing friction between moving surfaces comprising the step of contacting the surfaces with the lubricant or with the ethylene copolymer.

The ethylene copolymer is liquid, which usually means that it is liquid at room temperature, e.g. at 25° C.

The ethylene copolymers are usually not crystalline, so that in general no crystallization commencement temperature,  $T_{CC}$ , is measurable at  $T > 15^\circ C$ . with differential scanning calorimetry. Usually, a melt flow index cannot be determined with ethylene copolymers.

The ethylene copolymer may have a pour point below 25° C., preferably below 20° C., and in particular below 15° C. In another form the ethylene copolymer may have a pour point below 10° C., preferably below 5° C., and in particular below 0° C. The pour point may be determined according to ASTM D 97.

In one form the ethylene copolymer is considered liquid when its pour point is below 25° C., preferably below 20° C., and in particular below 15° C.

The ethylene copolymer may be clear liquid at room temperature, e.g. at 25° C. Typically, in a clear liquid no turbidity is visible.

The ethylene copolymer may have a cloud point of below 25° C., preferably below 20° C., and in particular below 15° C. The cloud point may be determined according to ISO 3015.

## 2

The ethylene copolymer may be miscible with a polyaliphatic olefin having a kinematic viscosity at 100° C. of about 6 cSt. This miscibility may be determined in a weight ratio of 50:50 at room temperature, e.g. 25° C. for 24 h.

5 The ethylene copolymer may have a viscosity index of at least 100, preferably at least 120, and in particular of at least 180. The viscosity index may be determined according to ASTM D2270.

10 The ethylene copolymer may have a kinematic viscosity at 40° C. from 200 to 30 000 mm<sup>2</sup>/s (cSt), preferably from 500 to 10 000 mm<sup>2</sup>/s, and in particular from 1000 to 5000 mm<sup>2</sup>/s. The kinematic viscosity may be determined according to ASTM D445.

15 In another form the ethylene copolymer may have a kinematic viscosity at 40° C. from 700 to 4000 mm<sup>2</sup>/s (cSt), preferably from 1000 to 3000 mm<sup>2</sup>/s, and in particular from 1200 to 2500 mm<sup>2</sup>/s.

20 In another form the ethylene copolymer may have a kinematic viscosity at 40° C. from 5000 to 50 000 mm<sup>2</sup>/s (cSt), preferably from 10 000 to 35 000 mm<sup>2</sup>/s, and in particular from 15 000 to 30 000 mm<sup>2</sup>/s.

25 The ethylene copolymer may have a kinematic viscosity at 100° C. from 10 to 5000 mm<sup>2</sup>/s (cSt), preferably from 30 to 3000 mm<sup>2</sup>/s, and in particular from 50 to 2000 mm<sup>2</sup>/s.

30 In another form the ethylene copolymer may have a kinematic viscosity at 100° C. from 50 to 500 mm<sup>2</sup>/s (cSt), preferably from 80 to 350 mm<sup>2</sup>/s, and in particular from 100 to 200 mm<sup>2</sup>/s.

35 In another form the ethylene copolymer may have a kinematic viscosity at 100° C. from 200 to 3000 mm<sup>2</sup>/s (cSt), preferably from 700 to 2500 mm<sup>2</sup>/s, and in particular from 800 to 2100 mm<sup>2</sup>/s.

40 In another form the ethylene copolymer may have a kinematic viscosity at 100° C. from 500 to 10 000 mm<sup>2</sup>/s (cSt), preferably from 900 to 5000 mm<sup>2</sup>/s, and in particular from 1200 to 4000 mm<sup>2</sup>/s.

45 The ethylene copolymer has usually a weight-average molecular weight  $M_w$  in the range up to 35 000 g/mol, preferably up to 30 000 g/mol, and in particular up to 25 000 g/mol. In another form the  $M_w$  is in the range up to 70 000 g/mol, preferably up to 50 000 g/mol, and in particular up to 40 000 g/mol.

50 In another form the ethylene copolymer has usually a weight-average molecular weight  $M_w$  in the range from 1000 to 30 000 g/mol, preferably from 1500 to 25 000 g/mol, and in particular from 3000 to 25000 g/mol.

55 In another form the ethylene copolymer has usually a weight-average molecular weight  $M_w$  in the range from 1 000 to 25 000 g/mol, preferably from 2 000 to 20 000 g/mol, and in particular from 3000 to 15 000 g/mol.

60 In another form the ethylene copolymer has usually a weight-average molecular weight  $M_w$  in the range from 8 000 to 35 000 g/mol, preferably from 10 000 to 30 000 g/mol, and in particular from 12 000 to 25 000 g/mol.

The ethylene copolymer has usually a number-average molecular weight  $M_n$  in the range up to 12000 g/mol, preferably up to 10000 g/mol, and in particular up to 7000 g/mol. In another form the  $M_n$  is in the range up to 25000 g/mol, preferably up to 15000 g/mol, and in particular up to 13000 g/mol.

65 In another form the ethylene copolymer has usually a number-average molecular weight  $M_n$  in the range from 1000 to 12000 g/mol, preferably from 1200 to 9000 g/mol, and in particular from 1500 to 7000 g/mol. The  $M_w$  and  $M_n$  may be determined by GPC on calibrated columns.

In another form the ethylene copolymer has usually a number-average molecular weight  $M_n$  in the range from

1000 to 10000 g/mol, preferably from 1500 to 8000 g/mol, and in particular from 1700 to 5000 g/mol.

In another form the ethylene copolymer has usually a number-average molecular weight  $M_n$  in the range from 2000 to 15 000 g/mol, preferably from 3500 to 10 000 g/mol, and in particular from 4000 to 7000 g/mol.

The ethylene copolymer has usually a polydispersity ( $M_w/M_n$ ) of at least 1, preferably in the range from 1.3 to 5, more preferably from 1.5 to 4, and most preferably from 1.8 to 3.8.

In another form the ethylene copolymer has usually a polydispersity in the range from 1.3 to 3.5, more preferably from 1.5 to 3.3, and most preferably from 1.9 to 3.0.

In another form the ethylene copolymer has usually a polydispersity in the range from 2.7 to 4.5, more preferably from 3.0 to 4.0, and most preferably from 3.2 to 3.8.

The liquid ethylene copolymer comprises in polymerized form 20 to 60 wt %, preferably 25 to 55 wt %, and in particular 30 to 50 wt % of ethylene.

In another form the liquid ethylene copolymer comprises in polymerized form 25 to 45 wt %, preferably 27 to 40 wt %, and in particular 30 to 38 wt % of ethylene.

In another form the liquid ethylene copolymer comprises in polymerized form 32 to 55 wt %, preferably 36 to 50 wt %, and in particular 40 to 46 wt % of ethylene.

In another form the liquid ethylene copolymer comprises in polymerized form at least 35, 40, 45, 50, 55, 60, 65, 70, 75, or 80 mol % of ethylene. In another form the liquid ethylene copolymer comprises in polymerized form 35 to 95 mol %, preferably 45 to 40 mol %, and in particular 55 to 88 mol % of ethylene. In another form the liquid ethylene copolymer comprises in polymerized form 60 to 95 mol %, preferably 65 to 40 mol %, and in particular 70 to 88 mol of ethylene.

The liquid ethylene copolymer comprises in polymerized form at least 20 wt %, preferably at least 40 wt %, and in particular at least 50 wt % of the acrylate. The ethylene copolymer may comprise in polymerized form 30 to 80 wt %, preferably 40 to 75 wt %, and in particular 50 to 75 wt % of the acrylate. In another form the liquid ethylene copolymer comprises in polymerized form at least 20, 25, 30, 35, 40, 45, 50, or 55 wt % of the acrylate. In another form the liquid ethylene copolymer comprises in polymerized form less than 80, 75, 70, 65, 60, 55, or 50 wt % of the acrylate.

In another form the liquid ethylene copolymer may comprise in polymerized form at least 5 mol %, preferably at least 10 mol %, and in particular at least 15 mol % of the acrylate. In another form the liquid ethylene copolymer may comprise in polymerized form at least 5, 10, 15, 20, 25, 30, or 35 mol % of the acrylate. In another form the liquid ethylene copolymer may comprise in polymerized form less than 20, 25, 30, 35, 40, or 45 mol % of the acrylate. In another form the ethylene copolymer may comprise in polymerized form 5 to 50 mol %, preferably 10 to 45 mol %, and in particular 15 to 40 mol % of the acrylate.

The wt % or the mol % of the monomers, which are present in polymerized form in the ethylene copolymer, usually refers to the total amount of monomers which are present in polymerized form in the ethylene copolymer. Other compounds, such as radical starters or chain transfer agents, may be incorporated in the ethylene copolymer, but they are usually not considered for this calculation.

Usually, the sum of the wt % of ethylene and the acrylate (e.g. the polar and the unpolar acrylate) and optionally the further monomer is up to 100 wt %, preferably 80 to 100 wt %, in particular 95 to 100 wt %. In another form the sum of

the wt % of ethylene and the acrylate is 100 wt %. Usually, the sum of the mol % of ethylene and the acrylate (e.g. the polar and the unpolar acrylate) and optionally the further monomer is up to 100 mol %, preferably 80 to 100 mol %, in particular 95 to 100 mol %. In another form the sum of the wt % of ethylene and the acrylate is 100 mol %. The wt % or the mol % of ethylene and the acrylate (and optionally the further monomers) in the ethylene copolymer may be determined by H-NMR.

- 10 In one form the ethylene copolymer comprises in polymerized form  
25 to 55 wt % of ethylene, and  
at least 40 wt % of the acrylate, such as 40 to 75 wt %,  
and in particular 50 to 75 wt %.
- 15 In another form the ethylene copolymer comprises in polymerized form  
30 to 50 wt % of ethylene, and  
at least 50 wt % of the acrylate, such as 50 to 75 wt %.  
In another form the ethylene copolymer comprises in polymerized form  
25 to 55 wt % of ethylene,  
at least 20 wt % of the polar acrylate, and  
at least 15 wt % of the unpolar acrylate.
- 20 In another form the ethylene copolymer comprises in polymerized form  
20 to 60 wt % of ethylene,  
20 to 50 wt % of the polar acrylate, and  
15 to 40 wt % of the unpolar acrylate.  
In another form the ethylene copolymer comprises in polymerized form  
30 to 50 wt % of ethylene,  
25 to 50 wt % of the polar acrylate, and  
20 to 40 wt % of the unpolar acrylate.
- 25 In another form the ethylene copolymer comprises in polymerized form  
25 to 55 wt % of ethylene,  
at least 20 wt % of the polar acrylate which is selected  
from  $C_1$ - $C_4$  alkyl (meth)acrylate, and  
at least 15 wt % of the unpolar acrylate which is selected  
from  $C_6$ - $C_{22}$  alkyl (meth)acrylate.
- 30 In another form the ethylene copolymer comprises in polymerized form  
30 to 50 wt % of ethylene,  
20 to 50 wt % of the polar acrylate which is selected from  
 $C_1$ - $C_4$  alkyl (meth)acrylate, and  
15 to 40 wt % of the unpolar acrylate which is selected  
from  $C_6$ - $C_{22}$  alkyl (meth)acrylate.
- 35 In another form the ethylene copolymer comprises in polymerized form  
25 to 55 wt % of ethylene,  
at least 20 wt % of the polar acrylate which is selected  
from  $C_3$ - $C_4$  alkyl (meth)acrylate, and  
at least 15 wt % of the unpolar acrylate which is selected  
from  $C_8$ - $C_{14}$  alkyl (meth)acrylate.
- 40 In another form the ethylene copolymer comprises in polymerized form  
30 to 50 wt % of ethylene,  
20 to 50 wt % of the polar acrylate which is selected from  
 $C_3$ - $C_4$  alkyl (meth)acrylate, and  
15 to 40 wt % of the unpolar acrylate which is selected  
from  $C_6$ - $C_{12}$  alkyl (meth)acrylate.
- 45 In another form the ethylene copolymer comprises in polymerized form  
25 to 55 wt % of ethylene,  
at least 20 wt % of the polar acrylate which is selected from  
 $C_3$ - $C_4$  alkyl (meth)acrylate, and  
at least 15 wt % of the unpolar acrylate which is selected  
from  $C_8$ - $C_{14}$  alkyl (meth)acrylate.
- 50 In another form the ethylene copolymer comprises in polymerized form  
30 to 50 wt % of ethylene,  
20 to 50 wt % of the polar acrylate which is selected from  
 $C_3$ - $C_4$  alkyl (meth)acrylate, and  
at least 15 wt % of the unpolar acrylate which is selected  
from  $C_8$ - $C_{12}$  alkyl (meth)acrylate.
- 55 In another form the ethylene copolymer comprises in polymerized form  
30 to 50 wt % of ethylene,  
20 to 50 wt % of the polar acrylate which is selected from  
 $C_3$ - $C_4$  alkyl (meth)acrylate, and  
at least 15 wt % of the unpolar acrylate which is selected  
from  $C_8$ - $C_{12}$  alkyl (meth)acrylate.
- 60 In another form the ethylene copolymer comprises in polymerized form  
30 to 50 wt % of ethylene,  
20 to 50 wt % of the polar acrylate which is selected from  
 $C_3$ - $C_4$  alkyl (meth)acrylate, and  
15 to 40 wt % of the unpolar acrylate which is selected  
from  $C_8$ - $C_{12}$  alkyl (meth)acrylate.
- 65 The acrylate is selected from  $C_1$ - $C_{22}$  alkyl (meth)acrylate, preferably from  $C_1$ - $C_{22}$  alkyl acrylate. The acrylate may comprise at least one (meth)acrylate, such as one, two or three (meth)acrylates. The acrylate is preferably selected from  $C_2$ - $C_{20}$  alkyl (meth)acrylate, and in particular from selected from  $C_3$ - $C_{18}$  alkyl (meth)acrylate. The acrylate is

preferably selected from branched C<sub>2</sub>-C<sub>20</sub> alkyl (meth)acrylate, and in particular from selected from branched C<sub>3</sub>-C<sub>18</sub> alkyl (meth)acrylate. In another form the acrylate is preferably selected from C<sub>2</sub>-C<sub>20</sub> alkyl acrylate, and in particular from selected from C<sub>3</sub>-C<sub>18</sub> alkyl acrylate. In another form the acrylate is preferably selected from branched C<sub>2</sub>-C<sub>20</sub> alkyl acrylate, and in particular from selected from branched C<sub>3</sub>-C<sub>18</sub> alkyl acrylate. In a preferred form the acrylate is 2-ethylhexyl acrylate.

The term "(meth)acrylate" refers to esters or acrylic acid, methacrylic acid, or mixtures thereof. Preferably, the acrylate is selected from C<sub>1</sub>-C<sub>22</sub> alkyl acrylate, in particular from C<sub>3</sub>-C<sub>18</sub> alkyl acrylates.

The C<sub>1</sub>-C<sub>22</sub> alkyl group of the C<sub>1</sub>-C<sub>22</sub> alkyl (meth)acrylate (preferably of the the C<sub>1</sub>-C<sub>22</sub> alkyl acrylate) may be saturated or unsaturated (preferably saturated), branched, cyclic or linear (preferably linear or branched) or mixtures thereof, such as methyl, ethyl, n-propyl, isopropyl, n-butyl, isobutyl, sec-butyl, tert-butyl, n-pentyl, isopentyl, sec-pentyl, neopen-tyl, 1,2-dimethyl-propyl, isoamyl, n-hexyl, isohexyl, sec-hexyl, cyclo-hexyl, n-heptyl, n-octyl, isoctyl, 2-ethylhexyl, n-nonyl, 2-propylheptyl, n-decyl, undecyl, dodecyl, tridecyl, 15 tetrade cyl, pentadecyl, hexadecyl, heptadecyl, octadecyl, 2-butyl octyl, 2-pentyl nonyl, 2-hexyl decyl, isohexyl, isoheptyl, isoctyl, isononyl, isodecyl, isoundecyl, isododecyl, 25 isotridecyl, isotetradecyl, isopentadecyl, isohexadecyl, isohexadecyl, isooctadecyl, and mixtures thereof.

The acrylate may comprise a polar acrylate and an unpo-  
lar acrylate. Preferably, the acrylate comprises

a polar acrylate selected from C<sub>1</sub>-C<sub>5</sub> alkyl (meth)acrylate (preferably C<sub>1</sub>-C<sub>5</sub> alkyl acrylate), and

an unpolar acrylate selected from C<sub>6</sub>-C<sub>22</sub> alkyl (meth)acrylate (preferably C<sub>6</sub>-C<sub>22</sub> alkyl acrylate).

The polar acrylate may be methyl (meth)acrylate, ethyl (meth)acrylate, n-propyl (meth)acrylate, or n-butyl (meth)acrylate, wherein n-butyl acrylate is preferred.

The unpolar acrylate may be preferably selected from C<sub>8</sub>-C<sub>18</sub> alkyl (meth)acrylate, and in particular from C<sub>8</sub>-C<sub>12</sub> alkyl (meth)acrylate. In another form the unpolar acrylate may be preferably selected from branched C<sub>8</sub>-C<sub>18</sub> alkyl (meth)acrylate, and in particular from branched C<sub>8</sub>-C<sub>12</sub> alkyl (meth)acrylate, such as 2-ethylhexyl acrylate.

Examples of the unpolar acrylate are (meth)acrylates of n-octyl, isoctyl, 2-ethylhexyl, n-nonyl, 2-propylheptyl, n-decyl, undecyl, dodecyl, tridecyl, tetrade cyl, pentadecyl, hexadecyl, heptadecyl, octadecyl, 2-butyl octyl, 2-pentyl nonyl, 2-hexyl decyl, isohexyl, isoheptyl, isoctyl, isononyl, isodecyl, isoundecyl, isododecyl, isotridecyl, isotetradecyl, isopentadecyl, isohexadecyl, isoheptadecyl, isooctadecyl and mixtures thereof.

More preferably, the polar acrylate is selected from C<sub>3</sub>-C<sub>4</sub> alkyl (meth)acrylate, and the unpolar acrylate selected from C<sub>8</sub>-C<sub>22</sub> alkyl (meth)acrylate (e.g. branched C<sub>8</sub>-C<sub>22</sub> alkyl (meth)acrylate).

In particular, the polar acrylate is selected from C<sub>3</sub>-C<sub>4</sub> alkyl acrylate, and the unpolar acrylate selected from C<sub>8</sub>-C<sub>22</sub> alkyl acrylate.

The weight ratio of the unpolar acrylate to the polar acrylate may be from 10:90 to 70:30, preferably from 20:80 to 65:35, and in particular from 30:70 to 60:40.

The ethylene copolymer may comprise in polymerized form further monomers beside ethylene and the acrylate, such as up to 10 wt %, preferably up to 4 wt %, and in particular up to 2 wt % of all monomers. Preferably, the ethylene copolymer is free of further monomers beside the ethylene and the acrylate. In another form the ethylene copolymer may comprise less than 2 wt %, preferably less

than 1 wt %, and in particular less than 0.3 wt % further monomers. In another form the ethylene copolymer may comprise in polymerized form less than 2 mol %, preferably less than 1 mol %, and in particular less than 0.5 mol % further monomers.

Examples for further monomers are

vinyl aromatic compounds, such as styrene, alpha-methyl styrene, vinyl toluene or p-(tert-butyl) styrene;

acrylamide and methacrylamide;

maleic acid and the imides and C<sub>1</sub> to C<sub>14</sub>-alkyl or di alkyl esters thereof;

fumaric acid and the imides and C<sub>1</sub> to C<sub>14</sub>-alkyl or di alkyl esters thereof;

itaconic acid and the imides and C<sub>1</sub> to C<sub>10</sub>-alkyl esters thereof;

acrylonitrile and methacrylonitrile;

acrylates and methacrylates with functionalized chain such as dimethylaminoethyl methacrylate, dimethylaminoethyl methacrylate, diethylaminoethyl methacrylate, dimethylaminoethyl acrylate, dimethylaminopropyl acrylate, diethylaminoethyl acrylate, diethylaminopropyl acrylate, tert-butylaminoethyl methacrylate, glycidyl methacrylate, phenoxyethyl acrylate, phenoxyethyl methacrylate, 2-morpholinoethyl methacrylate, hydroxyethyl methacrylate, hydroxypropyl methacrylate;

acrylamide derivatives such as N,N-dimethylaminopropyl methacrylamide, N,N-dimethylaminopropyl acrylamide, N,N-dimethylacrylamide, N,N-diethylacrylamide; vinyl derivatives such as vinylimidazol, vinylpyrrolidone, vinylformamide, vinyl ethers, propylvinyl ether, butylvinyl ether and cyclohexylvinyl ether.

Other suitable further monomers are C<sub>24</sub>-C<sub>40</sub> alkyl(meth)acrylates, which are preferably branched, such as (meth)acrylates of 2-decyl-tetradecanol, 2-dodecyl-hexadecanol, tetradecyl-octadecanol.

Other suitable further monomers are polyolefin-based macromonomers, preferably the macromonomers according to WO 2018/024563, such as macromonomers of the following formula (III)



wherein R<sup>1</sup> to R<sup>5</sup> are each independently selected from the group consisting of H, C<sub>1</sub>-C<sub>20</sub>-Alkyl, C<sub>1</sub>-C<sub>20</sub>-Alkoxy and C<sub>8</sub>-C<sub>3500</sub>-Polyisobutyl and C<sub>8</sub>-C<sub>3500</sub>-Polyisobut enyl, R is a 2 to 10 carbon atoms comprising alkylene group, R<sup>6</sup> is hydrogen or methyl, R<sup>7</sup> is hydrogen, methyl or COOR<sup>8</sup>, R<sup>8</sup> is hydrogen or C<sub>1</sub>-C<sub>20</sub>-alkyl, and n is a positive integer from 1 to 50, with the proviso that at least of the residues R<sup>1</sup> to R<sup>5</sup> is a C<sub>8</sub>-C<sub>3500</sub>-polyisobutyl or C<sub>8</sub>-C<sub>3500</sub>-polyisobut enyl.

In another form the further monomers are non-ionic monomers.

In another form the ethylene copolymer may be free of further monomers which are vinylester of the formula (I) in polymerized form



(I)

where  $R^c$ ,  $R^d$ , and  $R^e$  are each independently H or  $C_1$ - $C_4$ -alkyl, and  $R^f$  is  $C_1$ - $C_{20}$  alkyl. A suitable vinyl ester of the formula (I) is vinyl acetate. In another form the ethylene copolymer comprises less than 2 mol %, less than 1.5 mol %, less than 1.0 mol %, less than 0.5 mol % or less than 0.1 mol % of the vinylester of the formula (I), such as vinyl acetate. In another form the ethylene copolymer may be free of vinyl derivatives such as vinylester.

In another form the ethylene copolymer may comprise less than 5 wt %, preferably less than 1 wt %, and in particular less than 0.5 of an alkyl methacrylate in polymerized form (for example the ethylene copolymer is free of alkyl methacrylates) and the acrylate is selected from C1-022 alkyl acrylate.

In another form the ethylene copolymer may be free of further monomers in polymerized form, which comprise a functional group, such as a functional group selected from carboxylic acid, sulfonic acid, phosphonic acid, amino, amide, imide, hydroxyl, and cyano. In another form the ethylene copolymer may comprise less than 5 wt %, preferably less than 1 wt %, and in particular less than 0.5 wt % further monomers in polymerized form, which comprise a functional group.

In another form the ethylene copolymer may be free of further monomers which are vinylester of the formula (I) in polymerized form, and of further monomers in polymerized form, which comprise functional groups.

In another form the ethylene copolymer is free of further monomers in polymerized form, which comprise an ionic group (e.g. anionic, cationic, or zwitter ionic), such as a carboxylic acid, sulfonic acid, or phosphonic acid. In another form the ethylene copolymer may comprise less than 5 wt %, preferably less than 1 wt %, and in particular less than 0.5 wt % further monomers in polymerized form, which comprise an ionic group.

In another form the ethylene copolymer is free of further monomers in polymerized form, which comprise an acidic group, such as maleic acid, fumaric acid, itaconic acid, acrylic acid, and methacrylic acid. In another form the ethylene copolymer may comprise less than 5 wt %, preferably less than 1 wt %, and in particular less than 0.5 wt % further monomers in polymerized form, which comprise an acidic group, such as maleic acid, fumaric acid, itaconic acid, acrylic acid, and methacrylic acid. In another form the ethylene copolymer is free of acrylic acid and/or methacrylic acid in polymerized form. In another form the ethylene copolymer may comprise less than 5 wt %, preferably less than 1 wt %, and in particular less than 0.5 wt % of acrylic acid and/or methacrylic acid in polymerized form.

In another form the ethylene copolymer is free of further monomers in polymerized form, which comprise a hydroxyl group, such as hydroxalkyl (meth)acrylates. In another form the ethylene copolymer may comprise less than 5 wt %, preferably less than 1 wt %, and in particular less than 0.5 wt % further monomers in polymerized form, which comprise a hydroxyl group, such as hydroxalkyl (meth)acry-

lates. In another form the ethylene copolymer may be free of esters of unsaturated carboxylic acids in polymerized form containing at least one free hydroxyl group located in the part of the molecule derived from the alcohol.

5 The ethylene copolymer is usually obtainable by a continuous high-pressure polymerization process where a monomer feed comprising the ethylene and the acrylate is polymerized in the presence (e.g. of at least 2 wt %) of a chain transfer agent.

10 The polymerization process is usually a continuous process, which usually means that there is a continuous feed of starting materials (e.g. the monomer feed) and a continuous output of the polymeric product. The polymerization process may continue for at least 3 h, preferably at least 24 h, and in particular at least 72 h.

15 The polymerization process may be carried out in stirred high-pressure autoclaves, hereinafter also referred to as high-pressure autoclaves, or in high-pressure tube reactors, hereinafter also referred to as tube reactors. Preference is given to the high-pressure autoclaves, which may have a length/diameter ratio in the range from 5:1 to 30:1, preferably from 10:1 to 20:1.

20 The polymerization process may be carried out at a pressure in the range from 1000 to 4000 bar, preferably from 1200 to 2500 bar, and particularly 1600 to 2000 bar. Conditions of this type will hereinafter also be referred to as high-pressure. The pressure can change during the polymerization.

25 The polymerization process may be carried out at a reaction temperature in the range of 150 to 300°C, preferably 170 to 250°C, and in particular 190 to 230°C.

30 The monomer feed comprises usually the ethylene and the acrylate and optionally the chain transfer agent. Preferably, the monomer feed consists only of the ethylene and the acrylate and optionally the further monomer.

35 The monomer feed is usually polymerized, wherein the ethylene and the acrylate, and optionally the further monomer and optionally the chain transfer agent can be mixed before, during, or after entering the high-pressure autoclaves or the high-pressure tube reactors. Preferably, the monomer feed is polymerized, wherein the ethylene and the acrylate and optionally the further monomer are mixed before entering the high-pressure autoclaves. Typically, the polymerization process takes place in the polymerization zone, which is usually inside the high-pressure autoclave or the high-pressure tube reactor.

40 Preferably, the monomer feed is free of the initiator. Preferably, the monomer feed is free of the chain transfer agent.

45 The monomer feed may comprise the ethylene and the acrylate and optionally the further monomer in amounts which are suitable to arrive at the desired monomer amounts in the ethylene copolymer.

50 Usually, the monomer feed comprises at least 30 wt %, preferably at least 40 wt %, and in particular at least 50 wt % of ethylene, where the percentage is based on all monomers present in the monomer feed. In another form, the monomer feed comprises at least 30-90 wt %, preferably at least 40-80 wt %, and in particular at least 50-70 wt % of ethylene.

55 Usually, the monomer feed comprises at least 10 wt %, preferably at least 25 wt %, and in particular at least 35 wt % of acrylate, where the percentage is based on all monomers present in the monomer feed. In another form, the monomer feed comprises at least 10-70 wt %, preferably at least 20-60 wt %, and in particular at least 30-50 wt % of the acrylate.

The percentage of all monomers (e.g. ethylene, the acrylate and the further monomer) in the monomer feed usually sum up to 100%.

In another form the monomer feed comprises at least 30 wt % (e.g. at least 35, 40, 45, 50, 55, or 60 wt %) ethylene and at least 20 wt % (e.g. at least 25, 30, 35, 40 wt %) of the acrylate.

In another form the monomer feed comprises up to 90 wt % (e.g. up to 85, 80, 75, 70, or 65 wt %) ethylene and up to 70 wt % (e.g. up to 65, 60, 55, 50, 45, or 40 wt %) of the acrylate.

In another form the monomer feed comprises 30-90 wt % ethylene, 10-70 wt % of the acrylate, and optionally up to 20 wt % of further monomers, where the percentages of the monomers sum up to 100%.

In another form the monomer feed comprises 40-80 wt % ethylene, 20-60 wt % of the acrylate, and optionally up to 10 wt % of further monomers, where the percentages of the monomers sum up to 100%.

The conversion of the ethylene is usually around 15-70 wt %, preferably 25-55 wt % and in particular 30-45 wt %, based on the ethylene feed.

The input (e.g. kg monomer feed per hour) and the output (e.g. kg ethylene copolymer per hour) of the polymerization process depend on the size of the equipment. For example, a 1 liter autoclave may allow an input 6-25 kg/h monomer feed, or an output of 3-8 kg/h ethylene copolymer.

In a preferred form of the polymerization process the monomer feed is passed in the presence of the chain transfer agent at a temperature within the range from about 20 to 50° C., for example of 30° C., preferably continuously, into a stirred autoclave which is maintained at a pressure in the range from about 1200 to 2500 bar. The preferably continuous addition of initiator which is generally dissolved in a suitable solvent, for example isododecane or methylethylketone, keeps the temperature in the reactor at the desired reaction temperature, for example at from 150 to 280° C. The polymer obtained after the decompression of the reaction mixture may be then isolated.

Modifications to this method are of course possible and can be undertaken by those skilled in the art without unreasonable effort. For example, the monomers and the chain transfer agent can also be separately added into the reaction mixture using suitable pumps, or the reaction temperature can be varied during the process.

The percentage of the chain transfer agent can be based on the sum of the amounts of monomers (e.g. ethylene, the acrylate, optionally the further monomers) and the chain transfer agent. For example, a monomer feed of 15 kg/h ethylene and 3 kg/h acrylate and a feed of the chain transfer agent of 2 kg/h corresponds to the presence of 10 wt % of the chain transfer agent.

The monomer feed comprising the ethylene and the acrylate is usually polymerized in the presence of at least 1 wt %, or 2 wt %, preferably at least 5 wt %, and in particular at least 8 wt % of the chain transfer agent, e.g. in the polymerization zone. In another form the monomer feed comprising the ethylene and the acrylate may be polymerized in the presence of at least 1.1 wt %, or at least 1.3 wt %, or at least 1.5 wt %, or at least 1.7 wt %, or at least 2.1 wt %, or at least 2.3 wt %, or at least 2.5 wt %, or at least 3.0 wt %, or at least 3.5 wt %, or at least 4.0 wt %, or at least 4.5 wt %, or at least 5.0 wt %, or at least 5.5 wt %, or at least 6.0 wt %, or at least 6.5 wt %, or at least 7.0 wt %, or at least 8 wt %, or at least 9 wt %, or at least 10 wt % of the chain transfer agent.

In another form the monomer feed comprising the ethylene and the acrylate may be polymerized in the presence of up to 30 wt %, preferably up to 20 wt %, and in particular up to 15 wt % of the chain transfer agent.

In another form the monomer feed comprising the ethylene and the acrylate may be polymerized in the presence of 4 to 18 wt %, preferably 6 to 15 wt %, and in particular 9 to 13 wt % of the chain transfer agent.

In another form the monomer feed comprising the ethylene and the acrylate may be polymerized in the presence of 3.0 to 12 wt %, preferably 3.5 to 10 wt %, and in particular 4.0 to 8 wt % of the chain transfer agent.

Suitable chain transfer agents (also named regulator) in the sense of this invention are regulators which are terminating the growing of a polymer being incorporated as terminus of the polymer chain. Suitable regulators are saturated or unsaturated hydrocarbons, alcohols, thiols, ketones, aldehydes, amines, or hydrogen.

Among saturated and unsaturated hydrocarbons the chain transfer agents can be selected from pentane, hexane, cyclohexane, isododecane, propene, butene, pentene, cyclohexene, hexene, octene, decen and dodecen, and from aromatic hydrocarbons such as toluol, xylol, trimethylbenzene, ethylbenzene, diethylbenzene, triethylbenzene, mixtures thereof.

Suitable ketones or aldehydes as chain transfer agents are aliphatic aldehydes or aliphatic ketones, such as regulators of the formula II



or mixtures thereof.

$\text{R}^a$  and  $\text{R}^b$  are the same or different and are selected from hydrogen;

$\text{C}_1\text{-C}_6$ -alkyl such as methyl, ethyl, n-propyl, isopropyl, n-butyl, isobutyl, sec-butyl, tert-butyl, n-pentyl, isopentyl, sec-pentyl, neopentyl, 1,2-dimethylpropyl, isoamyl, n-hexyl, isohexyl, sec-hexyl; more preferably  $\text{C}_1\text{-C}_4$ -alkyl such as methyl, ethyl, n-propyl, isopropyl, n-butyl, isobutyl, sec-butyl and tert-butyl;

$\text{C}_3\text{-C}_{12}$ -cycloalkyl such as cyclopropyl, cyclobutyl, cyclopentyl, cyclohexyl, cycloheptyl, cyclooctyl, cyclo-nonyl, cyclodecyl, cycloundecyl and cyclododecyl; preference is given to cyclopentyl, cyclohexyl and cycloheptyl.

The  $\text{R}^a$  and  $\text{R}^b$  radicals may also be covalently bonded to one another to form a 4- to 13-membered ring. For example,  $\text{R}^a$  and  $\text{R}^b$  together may form the following alkylene groups:  $-(\text{CH}_2)_4-$ ,  $-(\text{CH}_2)_5-$ ,  $-(\text{CH}_2)_6-$ ,  $-(\text{CH}_2)_7-$ ,  $-\text{CH}(\text{CH}_3)-\text{CH}_2-\text{CH}_2-\text{CH}(\text{CH}_3)-$  or  $-\text{CH}(\text{CH}_3)-\text{CH}_2-\text{CH}_2-\text{CH}_2-\text{CH}(\text{CH}_3)-$ . Preferred ketones as chain transfer agents are acetone, methylethylketone, diethylketone and diamylketone.

Preferred aldehydes as chain transfer agents are acetaldehyde, propionaldehyde, butanal and pentanal.

Among alcohols the chain transfer agents are selected from the group consisting of methanol, ethanol, propanol, isopropanol, butanol and pentanol.

Among thiols the chain transfer agents maybe selected from mercaptoethanol to tetradecanethiol. In another form suitable thiols are organic thio compounds, such as primary, secondary, or tertiary aliphatic thiols, such as, ethanethiol,

## 11

n-propanethiol, 2-propanethiol, n-butanethiol, tert-butanethiol, 2-butanethiol, 2-methyl-2-propanethiol, n-pentanethiol, 2-pentanethiol, 3-pentanethiol, 2-methyl-2-butanethiol, 3-methyl-2-butanethiol, n-hexanethiol, 2-hexanethiol, 3-hexanethiol, 2-methyl-2-pantanethiol, 3-methyl-2-pantanethiol, 4-methyl-2-pantanethiol, 2-methyl-3-pantanethiol, 3-methyl-3-pantanethiol, 2-ethylbutanethiol, 2-ethyl-2-butanethiol, n-heptanethiol and its isomeric compounds, n-octanethiol and its isomeric compounds, n-nanonethiol and its isomeric compounds, n-decanethiol and its isomeric compounds, n-undecanethiol and its isomeric compounds, n-dodecanethiol and its isomeric compounds, n-tridecanethiol and its isomeric compounds, substituted thiols, such as 2-hydroxyethanethiol, aromatic thiols, such as benzenethiol, ortho-, meta-, or para-methylbenzenethiol, mercaptoalkanoic acid and derivatives thereof, such as 6-methylheptyl 3-mercaptopropionate or 2-ethylhexyl 2-mercaptopropanoate.

Among amines the chain transfer agents are selected from primary, secondary, or tertiary amines, such as dialkyl amines or trialkyl amines. Examples for amines are propyl amine, dipropyl amine, dibutyl amine, triethyl amine.

Preferred chain transfer agents are saturated or unsaturated hydrocarbons, aliphatic ketones, aliphatic aldehydes, or hydrogen, or mixtures thereof.

In another preferred form the chain transfer agents are propene, butene, pentene, propionaldehyde, methylethylketone, isododecane, or hydrogen, or mixtures thereof.

In another preferred form the chain transfer agents are propionaldehyde, methyl ethyl ketone, or hydrogen, or mixtures thereof.

In another preferred form the chain transfer agents are mixtures of propionaldehyde and/or methylethylketone and/or hydrogen.

In another preferred form the chain transfer agents is propionaldehyde. In another preferred form the chain transfer agents is a mixture of propionaldehyde and methylethylketone.

The chain transfer agents can be diluted with suitable solvents (e.g. hydrocarbons), preferably they are used without additional solvents.

The polymerization process is usually a free-radical polymerization, and usually initiated an initiator. Suitable initiators are organic peroxides, oxygen or azo compounds. Mixtures of a plurality of free-radical initiators are also suitable.

Suitable peroxides are didecanoyl peroxide, 2,5-dimethyl-2,5-di(2-ethylhexanoylperoxy)hexane, tert-amyl peroxyvalate, tert-amyl peroxy-2-ethylhexanoate, dibenzoyl peroxide, tert-butyl peroxy-2-ethylhexanoate, tert-butyl peroxydiethylacetate, tert-butyl peroxydiethylisobutyrate, 1,4-di(tert-butylperoxycarbonyl)cyclohexane as isomer mixture, tert-butyl perisononanoate, 1,1-di(tert-butylperoxy)-3,3,5-trimethylcyclohexane, 1,1-di(tert-butylperoxy)cyclohexane, methyl isobutyl ketone peroxide, tert-butyl peroxyisopropylcarbonate, 2,2-di(tert-butylperoxy)butane or tert-butyl peroxyacetate; tert-butyl peroxybenzoate, di-tert-amyl peroxide, dicumyl peroxide, the isomeric di-(tert-butylperoxyisopropyl)benzenes, 2,5-dimethyl-2,5-di-tert-butylperoxyhexane, tert-butyl cumyl peroxide, 2,5-dimethyl-2,5-di(tert-butylperoxy)hex-3-yne, di-tert-butylperoxide, 1,3-diisopropylbenzene monohydroperoxide, cumene hydroperoxide or tert-butyl hydroperoxide, or dimeric or trimeric ketone peroxides.

As azo compound azodicarboxylic esters, azodicarboxylic dinitriles are suitable, mention may be made by way of example of azobisisobutyronitrile ("AIBN").

## 12

Preferred initiators are selected from the group consisting of di-tert-butyl peroxide, tert-amyl peroxyvalate, tert-butyl peroxyvalat, tert-butyl peroxyisononanoate, tert-butyl peroxy-2-ethylhexanoate, 2,2-di(tert-butylperoxy)butane and mixtures thereof. Preferably tert-amyl peroxyvalate is used as initiator.

Initiators, e.g. organic peroxides, are often admixed with solvents to make them easier to handle. In a preferred form the initiator is introduced in the form of a solution in one or 10 more ketone(s) or hydrocarbons (especially olefins) which are liquid at room temperature. The initiator are preferably fed in as a 0.1-50% strength by weight solution, preferably a 0.5-20% strength by weight solution, in one or more hydrocarbons or one or more ketone(s) which are liquid at 15 room temperature or mixtures of hydrocarbons (e.g. olefins or aromatic hydrocarbons such as toluene, ethylbenzene, ortho-xylene, meta-xylene and para-xylene, also cycloaliphatic hydrocarbons such as cyclohexane and aliphatic C<sub>6</sub>-C<sub>16</sub>-hydrocarbons, either branched or unbranched, for example n-heptane, n-octane, isoctane, n-decane, n-dodecane and in particular isododecane), ketones (e.g. acetone, methyl isobutyl ketone, ethyl methyl ketone). In cases where the solvents for the initiator are also function as regulators (e.g. ketones), then the amount of such regulator is included 20 for calculating the wt % of the regulator in the monomer feed.

The amount of the initiator depends on the chemical nature of the initiator and can be adjusted by routine experiments. Typically, the initiator is present in 0.001 to 0.1 25 wt %, preferably 0.01 to 0.05 wt % based on the weight of the monomer feed.

The initiators employed herein can be introduced into the polymerization zone in any suitable manner, for example, by dissolving the initiator in a suitable solvent and injecting the 30 initiator solution directly into the polymerization zone. Alternatively, the initiator may be injected into the feed stream, either into the ethylene feed stream or the acrylate feed stream, prior to introduction thereof into the polymerization zone. The initiator can, for example, be fed in at the beginning, in the middle or after one third of the tube reactor. Initiator can also be fed in at a plurality of points on the tube reactor. In the autoclave it can be fed either in one point in the middle or twice: first in the upper part of the reactor and the second time either in the middle or in the bottom of the reactor. In addition three or more injections are possible.

The more preferable way to add monomers, chain transfer agent and solvents and other components in the process is mixing those together with ethylene in the middle pressure zone of 200-300 bar, in order increase the homogeneity of the mixtures of ethylene with the other components (called mixing within the compressor). Besides there is the possibility to add all liquids (chain transfer agents, monomers, solvents) directly to the high pressure zone of 1000-2200 45 bar; after the compression of ethylene (called mixing outside of the compressor). In addition both ways to add the liquids components can be used simultaneously.

The polymerization process may be followed by postpolymerization chemical reactions, such as a hydrogenation. The hydrogenation may be a homogeneous or heterogeneous catalytic hydrogenation. Usually, the hydrogenation is achieved with molecular hydrogen in the presence of a transition metal catalyst (e.g. based on RH, Co, Ni, Pd, or Pt), which may be dissolved in solvents or supported on inorganic supports.

The lubricant usually further comprises 60 a base oil selected from mineral oils, polyalphaolefins, polymerized and interpolymerized olefins, alkyl naph-

## 13

thalenes, alkylene oxide polymers, silicone oils, phosphate ester and carboxylic acid ester; and/or a lubricant additive.

In one form the lubricant further comprises a base oil selected from mineral oils, polyalphaolefins, polymerized and interpolymerized olefins, alkyl naphthalenes, alkylene oxide polymers, silicone oils, phosphate ester and carboxylic acid ester. In another form the lubricant usually further comprises a lubricant additive.

In one form the lubricant may comprise at least 10 wt %, preferably at least 30 wt % and in particular at least 60 wt % of the ethylene copolymer.

In another form the lubricant may comprise 10-99 wt %, preferably 30-95 wt % and in particular at least 60-95 wt % of the ethylene copolymer.

In another form the lubricant may comprise 1-90 wt %, preferably 5-50 wt % and in particular 20-50 wt % of the base oil.

In another form the lubricant may comprise at least 0.1 wt %, preferably at least 0.5 wt % and in particular at least 1 wt % of the ethylene copolymer.

In another form the lubricant may comprise 0.1-20 wt %, preferably 0.1-150 wt % and in particular at least 0.1-10 wt % of the ethylene copolymer.

In another form the lubricant may comprise 30-99.9 wt %, preferably 50-99 wt % and in particular 70-95 wt % of the base oil.

The lubricant may comprise up to 20 wt %, preferably up to 15 wt % and in particular up to 10 wt % of the lubricant additive.

In another form the lubricant may comprise 0.1-20 wt %, preferably 0.1-15 wt % and in particular at least 0.1-10 wt % of the lubricant additive.

Lubricants usually refers to composition which are capable of reducing friction between surfaces (preferably metal surfaces), such as surfaces of mechanical devices. A mechanical device may be a mechanism consisting of a device that works on mechanical principles. Suitable mechanical device are bearings, gears, joints and guidances. The mechanical device may be operated at temperatures in the range of -30°C to 80°C. Lubricants are usually specifically formulated for virtually every type of machine and manufacturing process. The type and concentration of base oils and/or lubricant additives used for these lubricants may be selected based on the requirements of the machinery or process being lubricated, the quality required by the builders and the users of the machinery, and the government regulation. Typically, each lubricant has a unique set of performance requirements. In addition to proper lubrication of the machine or process, these requirements may include maintenance of the quality of the lubricant itself, as well as the effect of the lubricant's use and disposal on energy use, the quality of the environment, and on the health of the user.

Typical lubricants are automotive lubricants (e.g. gasoline engine oils, diesel engine oils, gas engine oils, gas turbine oils, automatic transmission fluids, gear oils) and industrial lubricants (e.g. industrial gear oils, pneumatic tool lubricating oil, high temperature oil, gas compressor oil, hydraulic fluids, metalworking fluids).

Examples for lubricants are axle lubrication, medium and heavy duty engine oils, industrial engine oils, marine engine oils, automotive engine oils, crankshaft oils, compressor oils, refrigerator oils, hydrocarbon compressor oils, very low-temperature lubricating oils and fats, high temperature lubricating oils and fats, wire rope lubricants, textile machine oils, refrigerator oils, aviation and aerospace lubricants, aviation turbine oils, transmission oils, gas turbine

## 14

oils, spindle oils, spin oils, traction fluids, transmission oils, plastic transmission oils, passenger car transmission oils, truck transmission oils, industrial transmission oils, industrial gear oils, insulating oils, instrument oils, brake fluids, transmission liquids, shock absorber oils, heat distribution medium oils, transformer oils, fats, chain oils, minimum quantity lubricants for metalworking operations, oil to the warm and cold working, oil for water-based metalworking liquids, oil for neat oil metalworking fluids, oil for semi-synthetic metalworking fluids, oil for synthetic metalworking fluids, drilling detergents for the soil exploration, hydraulic oils, in biodegradable lubricants or lubricating greases or waxes, chain saw oils, release agents, molding fluids, gun, pistol and rifle lubricants or watch lubricants and food grade approved lubricants.

The lubricant has usually may have a kinematic viscosity at 40°C. of at least 10, 50, 100, 150, 200, 300, 400, 500, 600, 900, 1400, or 2000 mm<sup>2</sup>/s. In another form the lubricant has usually may have a kinematic viscosity at 40°C. from 200 to 30 000 mm<sup>2</sup>/s (cSt), preferably from 500 to 10 000 mm<sup>2</sup>/s, and in particular from 1000 to 5000 mm<sup>2</sup>/s.

The lubricant has usually may have a kinematic viscosity at 100°C. of at least 2, 3, 5, 10, 20, 30, 40, or 50 mm<sup>2</sup>/s. In another form the lubricant may have a kinematic viscosity at 100°C. from 10 to 5000 mm<sup>2</sup>/s (cSt), preferably from 30 to 3000 mm<sup>2</sup>/s, and in particular from 50 to 2000 mm<sup>2</sup>/s

The lubricant may have a viscosity index of at least 50, 75, 100, 120, 140, 150, 160, 170, 180, 190 or 200.

The lubricant is usually a lubricating liquid, lubricating oil or lubricating grease.

The base oil may selected from the group consisting of mineral oils (Group I, II or III oils), polyalphaolefins (Group IV oils), polymerized and interpolymerized olefins, alkyl naphthalenes, alkylene oxide polymers, silicone oils, phosphate esters and carboxylic acid esters (Group V oils). Preferably, the base oil is selected from Group I, Group II, Group III base oils according to the definition of the API, or mixtures thereof. Definitions for the base oils are the same as those found in the American Petroleum Institute (API) publication "Engine Oil Licensing and Certification System", Industry Services Department, Fourteenth Edition, December 1996, Addendum 1, December 1998. Said publication categorizes base oils as follows:

- a) Group I base oils contain less than 90 percent saturates (ASTM D 2007) and/or greater than 0.03 percent sulfur (ASTM D 2622) and have a viscosity index (ASTM D 2270) greater than or equal to 80 and less than 120.
- b) Group II base oils contain greater than or equal to 90 percent saturates and less than or equal to 0.03 percent sulfur and have a viscosity index greater than or equal to 80 and less than 120.
- c) Group III base oils contain greater than or equal to 90 percent saturates and less than or equal to 0.03 percent sulfur and have a viscosity index greater than or equal to 120.
- d) Group IV base oils contain polyalphaolefins. Polyalphaolefins (PAO) include known PAO materials which typically comprise relatively low molecular weight hydrogenated polymers or oligomers of alphaolefins which include but are not limited to C2 to about C32 alphaolefins with the C8 to about C16 alphaolefins, such as 1-octene, 1-decene, 1-dodecene and the like being preferred. The preferred polyalphaolefins are poly-1-octene, poly-1-decene, and poly-1-dodecene.

e) Group V base oils contain any base oils not described by Groups I to IV. Examples of Group V base oils include alkyl naphthalenes, alkylene oxide polymers, silicone oils, and phosphate esters.

Synthetic base oils include hydrocarbon oils and halo-substituted hydrocarbon oils such as polymerized and inter-polymerized olefins (e.g., polypropylenes, propylene-isobutylene copolymers, chlorinated polybutylenes, poly(1-hexenes), poly(1-octenes), poly(1-decenes)); alkylbenzenes (e.g., dodecylbenzenes, tetradecylbenzenes, dinonylbenzenes, di(2-ethylhexyl)benzenes); polyphenyls (e.g., biphenyls, terphenyls, alkylated polyphenols); and alkylated diphenyl ethers and alkylated diphenyl sulfides and derivative, analogs and homologs thereof.

Alkylene oxide polymers and interpolymers and derivatives thereof where the terminal hydroxyl groups have been modified by esterification, etherification, etc., constitute another class of known synthetic base oils. These are exemplified by polyoxyalkylene polymers prepared by polymerization of ethylene oxide or propylene oxide, and the alkyl and aryl ethers of polyoxyalkylene polymers (e.g., methyl-polyiso-propylene glycol ether having a molecular weight of 1000 or diphenyl ether of polyethylene glycol having a molecular weight of 1000 to 1500); and mono- and polycarboxylic esters thereof, for example, the acetic acid esters, mixed C3-C8 fatty acid esters and C13 oxo acid diester of tetraethylene glycol.

Silicon-based oils such as the polyalkyl-, polyaryl-, polyalkoxy- or polyaryloxysilicone oils and silicate oils comprise another useful class of synthetic base oils; such base oils include tetraethyl silicate, tetraisopropyl silicate, tetra-(2-ethylhexyl)silicate, tetra-(4-methyl-2-ethyl-hexyl) silicate, tetra-(p-tert-butyl-phenyl) silicate, hexa-(4-methyl-2-ethylhexyl)disiloxane, poly(methyl) siloxanes and poly (methylphenyl)siloxanes. Other synthetic base oils include liquid esters of phosphorous-containing acids (e.g., tricresyl phosphate, trioctyl phosphate, diethyl ester of decylphosphoric acid) and polymeric tetrahydrofurans.

Suitable lubricant additives may be selected from viscosity index improvers, polymeric thickeners, antioxidants, corrosion inhibitors, detergents, dispersants, anti-foam agents, dyes, wear protection additives, extreme pressure additives (EP additives), anti-wear additives (AW additives), friction modifiers, metal deactivators, pour point depressants.

The viscosity index improvers include high molecular weight polymers that increase the relative viscosity of an oil at high temperatures more than they do at low temperatures. Viscosity index improvers include polyacrylates, polymethacrylates, alkylmethacrylates, vinylpyrrolidone/methacrylate copolymers, poly vinylpyrrolidones, polybutenes, olefin copolymers such as an ethylene-propylene copolymer or a styrene-butadiene copolymer or polyalkene such as PIB, styrene/acrylate copolymers and polyethers, and combinations thereof. The most common VI improvers are methacrylate polymers and copolymers, acrylate polymers, olefin polymers and copolymers, and styrenebutadiene copolymers. Other examples of the viscosity index improver include polymethacrylate, polyisobutylene, alpha-olefin polymers, alpha-olefin copolymers (e.g., an ethylene-propylene copolymer), polyalkylstyrene, phenol condensates, naphthalene condensates, a styrenebutadiene copolymer and the like. Of these, polymethacrylate having a number average molecular weight of 10000 to 300000, and alpha-olefin polymers or alpha-olefin copolymers having a number average molecular weight of 1000 to 30000, particularly ethylene-alpha-olefin copolymers having a number average

molecular weight of 1000 to 10000 are preferred. The viscosity index increasing agents can be added and used individually or in the form of mixtures, conveniently in an amount within the range of from  $\geq 0.05$  to  $\geq 20.0\%$  by weight, in relation to the weight of the base stock.

Suitable (polymeric) thickeners include, but are not limited to, polyisobutenes (PIB), oligomeric co-polymers (OCPs), polymethacrylates (PMAs), copolymers of styrene and butadiene, or high viscosity esters (complex esters).

10 Antioxidants include phenolic antioxidants such as hindered phenolic antioxidants or non-phenolic oxidation inhibitors.

Useful phenolic antioxidants include hindered phenols. These phenolic antioxidants may be ashless (metal-free) 15 phenolic compounds or neutral or basic metal salts of certain phenolic compounds. Typical phenolic antioxidant compounds are the hindered phenolics which are the ones which contain a sterically hindered hydroxyl group, and these include those derivatives of dihydroxy aryl compounds in 20 which the hydroxyl groups are in the o- or p-position to each other. Typical phenolic antioxidants include the hindered phenols substituted with alkyl groups having 6 carbon atoms or more and the alkylene coupled derivatives of these hindered phenols. Examples of phenolic materials of this type 2-t-butyl-4-heptyl phenol; 2-t-butyl-4-octyl phenol; 2-t-butyl-4-dodecyl phenol; 2,6-di-t-butyl-4-heptyl phenol; 2,6-di-t-butyl-4-dodecyl phenol; 2-methyl-6-t-butyl-4-heptyl phenol; and 2-methyl-6-t-butyl-4-dodecyl phenol. Other useful hindered mono-phenolic antioxidants may include for 30 example hindered 2,6-di-alkyl-phenolic propionic ester derivatives. Bis-phenolic antioxidants may also be used in combination with the present invention. Examples of ortho-coupled phenols include: 2,2'-bis(4-heptyl-6-t-butyl-phenol); 2,2'-bis(4-octyl-6-t-butyl-phenol); and 2,2'-bis(4-dodecyl-6-t-butyl-phenol). Para-coupled bisphenols include for 35 example 4,4'-bis(2,6-di-t-butyl phenol) and 4,4'-methylene-bis(2,6-di-t-butyl phenol).

Non-phenolic oxidation inhibitors which may be used 40 include aromatic amine antioxidants and these may be used either as such or in combination with phenolics. Typical examples of non-phenolic antioxidants include: alkylated and non-alkylated aromatic amines such as aromatic mono-amines of the formula  $R^8R^9R^{10}N$ , where  $R^8$  is an aliphatic, aromatic or substituted aromatic group,  $R^9$  is an aromatic or 45 a substituted aromatic group, and  $R^{10}$  is H, alkyl, aryl or  $R^{11}S(O)_xR^{12}$ , where  $R^{11}$  is an alkylene, alkenylene, or alkylidene group,  $R^{12}$  is a higher alkyl group, or an alkenyl, aryl, or alkaryl group, and  $x$  is 0, 1 or 2. The aliphatic group  $R^8$  may contain from 1 to about 20 carbon atoms, and preferably contains from about 6 to 12 carbon atoms. The aliphatic group is a saturated aliphatic group. Preferably, both  $R^8$  and  $R^9$  are aromatic or substituted aromatic groups, and the aromatic group may be a fused ring aromatic group such as naphthyl. Aromatic groups  $R^8$  and  $R^9$  may be joined together 55 with other groups such as S.

Typical aromatic amines antioxidants have alkyl substituent groups of at least about 6 carbon atoms. Examples of 60 aliphatic groups include hexyl, heptyl, octyl, nonyl, and decyl. Generally, the aliphatic groups will not contain more than about 14 carbon atoms. The general types of amine antioxidants useful in the present compositions include diphenylamines, phenyl naphthylamines, phenothiazines, imidodibenzyls and diphenyl phenylene diamines. Mixtures of two or more aromatic amines are also useful. Polymeric 65 amine antioxidants can also be used. Particular examples of aromatic amine antioxidants useful in the present invention include: p,p'-dioctyldiphenylamine; t-octylphenyl-alpha-

naphthylamine; phenyl-alpha-naphthylamine; and p-oc-tylphenyl-alpha-naphthylamine. Sulfurized alkyl phenols and alkali or alkaline earth metal salts thereof also are useful antioxidants.

Corrosion inhibitors may include various oxygen-, nitrogen-, sulfur-, and phosphorus-containing materials, and may include metal-containing compounds (salts, organometallics, etc.) and nonmetal-containing or ashless materials. Corrosion inhibitors may include, but are not limited to, additive types such as, for example, hydrocarbyl-, aryl-, alkyl-, arylalkyl-, and alkylaryl-versions of detergents (neutral, overbased), sulfonates, phenates, salicylates, alcohulates, carboxylates, salixarates, phosphites, phosphates, thiophosphates, amines, amine salts, amine phosphoric acid salts, amine sulfonic acid salts, alkoxylated amines, etheramines, polyetheramines, amides, imides, azoles, diazoles, triazoles, benzotriazoles, benzothiadioles, mercaptobenzothiazoles, tolyltriazoles (TTZ-type), heterocyclic amines, heterocyclic sulfides, thiazoles, thiadiazoles, mercaptothiadiazoles, dimercaptothiadiazoles (DMTD-type), imidazoles, benzimidazoles, dithiobenzimidazoles, imidazolines, oxazolines, Mannich reactions products, glycidyl ethers, anhydrides, carbamates, thiocarbamates, dithiocarbamates, polyglycols, etc., or mixtures thereof.

Detergents include cleaning agents that adhere to dirt particles, preventing them from attaching to critical surfaces. Detergents may also adhere to the metal surface itself to keep it clean and prevent corrosion from occurring. Detergents include calcium alkylsalicylates, calcium alkylphenates and calcium alkylsulfonates with alternate metal ions used such as magnesium, barium, or sodium. Examples of the cleaning and dispersing agents which can be used include metal-based detergents such as the neutral and basic alkaline earth metal sulphonates, alkaline earth metal phenates and alkaline earth metal salicylates alkenylsuccinimide and alkenylsuccinimide esters and their borohydrides, phenates, salenius complex detergents and ashless dispersing agents which have been modified with sulphur compounds. These agents can be added and used individually or in the form of mixtures, conveniently in an amount within the range of from  $\geq 0.01$  to  $\leq 1.0$  by weight in relation to the weight of the base stock; these can also be high total base number (TBN), low TBN, or mixtures of high/low TBN.

Dispersants are lubricant additives that help to prevent sludge, varnish and other deposits from forming on critical surfaces. The dispersant may be a succinimide dispersant (for example N-substituted long chain alkenyl succinimides), a Mannich dispersant, an ester-containing dispersant, a condensation product of a fatty hydrocarbyl monocarboxylic acylating agent with an amine or ammonia, an alkyl amino phenol dispersant, a hydrocarbyl-amine dispersant, a polyether dispersant or a polyetheramine dispersant. In one embodiment, the succinimide dispersant includes a poly-isobutylene-substituted succinimide, wherein the poly-isobutylene from which the dispersant is derived may have a number average molecular weight of about 400 to about 5000, or of about 950 to about 1600. In one embodiment, the dispersant includes a borated dispersant. Typically, the borated dispersant includes a succinimide dispersant including a polyisobutylene succinimide, wherein the polyisobutylene from which the dispersant is derived may have a number average molecular weight of about 400 to about 5000. Borated dispersants are described in more detail above within the extreme pressure agent description.

Anti-foam agents may be selected from silicones, polyacrylates, and the like. The amount of anti-foam agent in the lubricant compositions described herein may range from

$\geq 0.001$  wt.-% to  $\leq 0.1$  wt.-% based on the total weight of the formulation. As a further example, an anti-foam agent may be present in an amount from about 0.004 wt.-% to about 0.008 wt.-%.

- 5 Suitable extreme pressure agent is a sulfur-containing compound. In one embodiment, the sulfur-containing compound may be a sulfurised olefin, a polysulfide, or mixtures thereof. Examples of the sulfurised olefin include a sulfurised olefin derived from propylene, isobutylene, pentene; an 10 organic sulfide and/or polysulfide including benzylsulfide; bis-(chlorobenzyl) disulfide; dibutyl tetrasulfide; di-tertiary butyl polysulfide; and sulfurised methyl ester of oleic acid, a sulfurised alkylphenol, a sulfurised dipentene, a sulfurised terpene, a sulfurised Diels-Alder adduct, an alkyl sulphenyl 15 N'N-dialkyl dithiocarbamates; or mixtures thereof. In one embodiment, the sulfurised olefin includes a sulfurised olefin derived from propylene, isobutylene, pentene or mixtures thereof. In one embodiment the extreme pressure additive sulfur-containing compound includes a dimercaptothiadiazole or derivative, or mixtures thereof. Examples of the dimercaptothiadiazole include compounds such as 2,5-dimercapto-1,3,4-thiadiazole or a hydrocarbyl-substituted 2,5-dimercapto-1,3,4-thiadiazole, or oligomers thereof. The oligomers of hydrocarbyl-substituted 2,5-dimercapto-1,3,4-thiadiazole typically form by forming a sulfur-sulfur bond between 2,5-dimercapto-1,3,4-thiadiazole units to form derivatives or oligomers of two or more of said thiadiazole units. Suitable 2,5-dimercapto-1,3,4-thiadiazole derived compounds include for example 2,5-bis(tert-nonyldithio)-1, 20 3,4-thiadiazole or 2-tert-nonyldithio-5-mercaptop-1,3,4-thiadiazole. The number of carbon atoms on the hydrocarbyl substituents of the hydrocarbyl-substituted 2,5-dimercapto-1,3,4-thiadiazole typically include 1 to 30, or 2 to 20, or 3 to 16. Extreme pressure additives include compounds containing boron and/or sulfur and/or phosphorus. The extreme pressure agent may be present in the lubricant compositions at 0 wt.-% to about 20 wt.-%, or at about 0.05 wt.-% to about 10.0 wt.-%, or at about 0.1 wt.-% to about 8 wt.-% of the lubricant composition.
- 25 30 35 40 Examples of anti-wear additives include organo borates, organo phosphites such as didodecyl phosphite, organic sulfur-containing compounds such as sulfurized sperm oil or sulfurized terpenes, zinc dialkyl dithiophosphates, zinc diaryl dithiophosphates, phosphosulfurized hydrocarbons and any combinations thereof.
- 45 Friction modifiers may include metal-containing compounds or materials as well as ashless compounds or materials, or mixtures thereof. Metal-containing friction modifiers include metal salts or metal-ligand complexes where the metals may include alkali, alkaline earth, or transition group metals. Such metal-containing friction modifiers may also have low-ash characteristics. Transition metals may include Mo, Sb, Sn, Fe, Cu, Zn, and others. Ligands may include hydrocarbyl derivative of alcohols, polyols, glycerols, partial ester glycerols, thiols, carboxylates, carbamates, thiocarbamates, dithiocarbamates, phosphates, thiophosphates, dithiophosphates, amides, imides, amines, thiazoles, thiadiazoles, dithiazoles, diazoles, triazoles, and other polar molecular functional groups containing effective amounts of O, N, S, or P, individually or in combination. In particular, Mo-containing compounds can be particularly effective such as for example Mo-dithiocarbamates, Mo(DTC), Mo-dithiophosphates, Mo(DTP), Mo-amines, Mo (Am), Mo-alcohates, Mo-alcohol-amides, and the like.
- 50 55 60 65 70 Ashless friction modifiers may also include lubricant materials that contain effective amounts of polar groups, for example, hydroxyl-containing hydrocarbyl base oils, glyc-

erides, partial glycerides, glyceride derivatives, and the like. Polar groups in friction modifiers may include hydrocarbyl groups containing effective amounts of O, N, S, or P, individually or in combination. Other friction modifiers that may be particularly effective include, for example, salts (both ash-containing and ashless derivatives) of fatty acids, fatty alcohols, fatty amides, fatty esters, hydroxyl-containing carboxylates, and comparable synthetic long-chain hydrocarbyl acids, alcohols, amides, esters, hydroxy carboxylates, and the like. In some instances, fatty organic acids, fatty amines, and sulfurized fatty acids may be used as suitable friction modifiers. Examples of friction modifiers include fatty acid esters and amides, organo molybdenum compounds, molybdenum dialkylthiocarbamates and molybdenum dialkyl dithiophosphates.

Suitable metal deactivators include benzotriazoles and derivatives thereof, for example 4- or 5-alkylbenzotriazoles (e.g. triazole) and derivatives thereof, 4,5,6,7-tetrahydrobenzotriazole and 5,5'-methylenebisbenzotriazole; Mannich bases of benzotriazole or triazole, e.g. 1-[bis(2-ethylhexyl) aminomethyl] triazole and 1-[bis(2-ethylhexyl) aminomethyl]benzotriazole; and alkoxy-alkylbenzotriazoles such as 1-(nonyloxymethyl)benzotriazole, 1-(1-butoxyethyl) benzotriazole and 1-(1-cyclohexyloxybutyl) triazole, and combinations thereof. Additional non-limiting examples of the one or more metal deactivators include 1,2,4-triazoles and derivatives thereof, for example 3-alkyl(or aryl)-1, 2,4-triazoles, and Mannich bases of 1,2,4-triazoles, such as 1-[bis(2-ethylhexyl) aminomethyl-1, 2,4-triazole; alkoxyalkyl-1, 2,4-triazoles such as 1-(1-butoxyethyl)-1, 2,4-triazole; and acylated 3-amino-1, 2,4-triazoles, imidazole derivatives, for example 4,4'-methylenebis(2-undecyl-5-methylimidazole) and bis[(N-methyl)imidazol-2-yl]carbinol octyl ether, and combinations thereof. Further non-limiting examples of the one or more metal deactivators include sulfur-containing heterocyclic compounds, for example 2-mercaptopbenzothiazole, 2,5-dimercapto-1, 3,4-thiadiazole and derivatives thereof; and 3,5-bis[di(2-ethylhexyl) aminomethyl]-1, 3,4-thiadiazolin-2-one, and combinations thereof. Even further non-limiting examples of the one or more metal deactivators include amino compounds, for example salicylidenepropylenediamine, salicylaminoguanidine and salts thereof, and combinations thereof. The one or more metal deactivators are not particularly limited in amount in the composition but are typically present in an amount of from about 0.01 to about 0.1, from about 0.05 to about 0.01, or from about 0.07 to about 0.1, wt.-% based on the weight of the composition. Alternatively, the one or more metal deactivators may be present in amounts of less than about 0.1, of less than about 0.7, or less than about 0.5, wt.-% based on the weight of the composition.

Pour point depressants (PPD) include polymethacrylates, alkylated naphthalene derivatives, and combinations thereof. Commonly used additives such as alkylaromatic polymers and polymethacrylates are also useful for this purpose. Typically, the treat rates range from 0.001 wt.-% to 1.0 wt.-%, in relation to the weight of the base stock.

Demulsifiers include trialkyl phosphates, and various polymers and copolymers of ethylene glycol, ethylene oxide, propylene oxide, or mixtures thereof.

The invention further relates to a method for reducing friction between moving surfaces (e.g. metal surfaces) comprising the step of contacting the surfaces with the lubricant or with the ethylene copolymer.

The friction may be determined by measuring the friction coefficient at 25% slide roll ratio (SRR) using mini-traction machine (MTM) measurements at 70° C. and 1 GPa.

The ethylene copolymer according to the invention may be used for many purposes in lubricants, e.g. for increasing the viscosity index of the lubricant, for thickening of the lubricant, for improving the coefficient of friction of the lubricant, for reducing wear, or as a base stock for the lubricant. The invention also related to a use of the ethylene copolymer for thickening of the lubricant.

## EXAMPLES

- 20 NBA: N-butyl acrylate,  
EHA: 2-Ethylhexyl acrylate, commercially available from BASF SE.  
PHA: 2-Propylheptyl acrylate, commercially available from BASF SE.  
25 LA: Lauryl acrylate (60:40 mixture of C12:014 alkyl acrylates)  
C17A: Heptadecyl acrylate, based on mixture of branched C17 alcanols, commercially available from BASF SE.

### Preparation of Copolymers

A high-pressure autoclave, of the type described in the literature (M. Buback et al, *Chem. Ing. Tech.* 1994, 66, 510-513) was used for continuous copolymerization

35 Ethylene was fed continuously into a first compressor until approx. 250 bar. Separately from this, the amount of the acrylate was also compressed continuously to an intermediate pressure of 250 bar and was mixed with the ethylene fed. The ethylene acrylate mixture was further compressed using a second compressor. The reaction mixture is brought to a 1 liter autoclave with pressure and temperatures given also according to Table 1. The desired temperature is controlled depending on the amount of initiator tert-amyl peroxypivalate in isodecane, which is introduced to the autoclave separately from the monomer feed (about 1000-1500 ml/h).

40 Separately from this, the amount of chain transfer agent propionaldehyde (PA) or methylethyl ketone (MEK) was first compressed to an intermediate pressure of 250 bar and then fed continuously into the high-pressure autoclave with the aid of a further compressor under the reaction pressure.

45 The output of the reactions in Table 1 was usually around 5-6 kg/h at a conversion of 30 to 45 wt % (based on ethylene feed). Details of the reaction conditions were summarized in Table 1 and the analytical data of the liquid ethylene copolymers are summarized in Table 2. The regulator feed in Table 1 refers to propionaldehyde if nothing else is indicated.

TABLE 1

| Preparation of liquid ethylene copolymers |          |            |             |                        |                       |                       |
|-------------------------------------------|----------|------------|-------------|------------------------|-----------------------|-----------------------|
| Ex.                                       | Monomers | P<br>[bar] | T<br>[° C.] | Ethylene<br>Feed       | Acrylate<br>Feed      | Regulator<br>Feed     |
| 1                                         | E-MA     | 1700       | 220         | 11820 g/h<br>60.8 wt % | 5035 g/h<br>25.9 wt % | 2600 g/h<br>13.4 wt % |

TABLE 1-continued

| Preparation of liquid ethylene copolymers |              |            |             |                        |                                                                                     |                                                      |
|-------------------------------------------|--------------|------------|-------------|------------------------|-------------------------------------------------------------------------------------|------------------------------------------------------|
| Ex.                                       | Monomers     | P<br>[bar] | T<br>[° C.] | Ethylene<br>Feed       | Acrylate<br>Feed                                                                    | Regulator<br>Feed                                    |
| 2                                         | E-EA         | 1700       | 220         | 11950 g/h<br>68.3 wt % | 3080 g/h<br>17.6 wt %                                                               | 2460 g/h<br>14.1 wt %                                |
| 3                                         | E-NBA        | 1700       | 220         | 11970 g/h<br>63 wt %   | 4986 g/h<br>26.2 wt %                                                               | 2049 g/h<br>10.8 wt %                                |
| 4                                         | E-EHA        | 1700       | 220         | 12040 g/h<br>58.5 wt % | 5961 g/h<br>29 wt %                                                                 | 2576 g/h<br>12.5 wt %                                |
| 5                                         | E-PHA        | 1700       | 220         | 12000 g/h<br>60.5 wt % | 5510 g/h<br>27.8 wt %                                                               | 2317 g/h<br>11.7 wt %                                |
| 6                                         | E-LA         | 1700       | 220         | 11920 g/h<br>59.8 wt % | 6130 g/h<br>31.4 wt %                                                               | 1500 g/h<br>7.6 wt %                                 |
| 7                                         | E-EHA-NBA    | 1800       | 220         | 12020 g/h<br>60.3 wt % | EHA: 2930 g/h<br>14.7 wt %<br>NBA: 2790 g/h<br>14.5 wt %                            | 1500 g/h<br>7.6 wt %                                 |
| 8                                         | E-LA-NBA     | 1800       | 220         | 12180 g/h<br>60.7 wt % | LA: 3250<br>16.2 g/h<br>NBA: 3130 g/h<br>15.6 wt %                                  | 1510 g/h<br>7.5 wt %                                 |
| 9                                         | E-LA-EHA-NBA | 1800       | 220         | 12030 g/h<br>61.6 wt % | LA: 2470 g/h<br>12.6 wt %<br>EHA: 500 g/h<br>2.6 wt %<br>NBA: 3000 g/h<br>15.4 wt % | 1540 g/h<br>7.9 wt %                                 |
| 10                                        | E-LA-NBA     | 1900       | 200         | 11890 g/h<br>76.3 wt % | LA: 1510 g/h<br>9.7 wt %<br>NBA: 1480 g/h<br>9.5 wt %                               | MEK: 350 g/h<br>2.2 wt %<br>PA: 350 g/h<br>2.2 wt %  |
| 11                                        | E-LA-NBA     | 1900       | 200         | 12120 g/h<br>74.6 wt % | LA: 1540 g/h<br>9.5 wt %<br>NBA: 1480 g/h<br>9.1 wt %                               | MEK: 910 g/h<br>5.6 wt %<br>PA: 200 g/h<br>1.2 wt %  |
| 12                                        | E-PHA-NBA    | 1700       | 220         | 11960 g/h<br>59.9 wt % | PHA: 3020 g/h<br>15.1 wt %<br>NBA: 3050 g/h<br>15.3 wt %                            | MEK: 1520 g/h<br>7.6 wt %<br>PA: 400 g/h<br>2.0 wt % |
| 13                                        | E-C17A-NBA   | 1700       | 220         | 11970 g/h<br>62.5 wt % | C17: 2010 g/h<br>10.5 wt %<br>NBA: 3960 g/h<br>20.7 wt %                            | 1210 g/h<br>6.3 wt %                                 |
| 14                                        | E-LA-NBA     | 2100       | 200         | 12030 g/h<br>77.4 wt % | LA: 1400 g/h<br>9.0 wt %<br>NBA: 1510 g/h<br>9.7 wt %                               | MEK: 300 g/h<br>1.9 wt %<br>PA: 300 g/h<br>1.9 wt %  |
| 15                                        | E-EHA        | 1900       | 200         | 12040 g/h              | 3000 g/h                                                                            | 300 g/h<br>2.0 wt %                                  |
| 16                                        | E-EHA        | 1900       | 200         | 12070 g/h              | 3000 g/h                                                                            | 400 g/h<br>2.6 wt %                                  |
| 17                                        | E-EHA        | 1900       | 200         | 12040 g/h              | 3000 g/h                                                                            | PA: 300 g/h<br>2.0 wt %<br>MEK: 80 g/h<br>0.5 wt %   |
| 18                                        | E-E-EHA-NBA  | 1900       | 200         | 12070 g/h              | EHA: 1250 g/h<br>NBA: 1250 g/h                                                      | 300 g/h<br>2.0 wt %                                  |

## Characterization of the Liquid Ethylene Copolymers

The molecular weight number distribution Mn and the molecular weight weight distribution Mw were determined via GPC. The polydispersity was calculated as PD=(Mw/Mn). The GPC analysis was made with a RI detector, a PLgel MIXED-B column (column temperature 35° C.) and THF with 0.1% trifluor acetic acid as elution medium. The calibration was done with very narrow distributed polystyrene standards from the Polymer Laboratories with a molecular weights M=from 580 until 6,870,000 g/mol.

The Cloud Point CP was determined according to ISO 3015. The Pour Point PP was determined according to ASTM D 97.

The results demonstrated that all ethylene copolymers were liquid at room temperature and had a pour point below 25° C.

The results further indicate that all ethylene copolymers tend to have good low temperature characteristics because of their low cloud point.

The amounts of monomers which are present in polymerized form in the polymer was determined by H-NMR.

TABLE 2

| Analytical data of copolymers |                |            |            |     |           |           |
|-------------------------------|----------------|------------|------------|-----|-----------|-----------|
| Ex. Monomers                  | Amounts [wt %] | Mn [g/mol] | Mw [g/mol] | PD  | PP [° C.] | CP [° C.] |
| 1 E-MA                        | 34-66          | 2250       | 4900       | 2.2 | 3         | -25       |
| 2 E-EA                        | 32-68          | 2380       | 5210       | 2.3 | -12       | -42       |
| 3 E-NBA                       | 33-67          | 2760       | 5290       | 2.2 | -30       | -19       |
| 4 E-EHA                       | 34-66          | 1990       | 4050       | 2.0 | -33       | -60       |
| 5 E-PHA                       | 35-65          | 1920       | 3850       | 2.0 | -33       | 5         |
| 6 E-LA                        | 37.5-62.5      | 3630       | 7940       | 2.2 | 6         | 18        |
| 7 E-EHA-NBA                   | 32-35-33       | 2670       | 6520       | 2.4 | -27       | -54       |
| E-LA-NBA                      | 35-32-33       | 2740       | 7490       | 2.7 | -9        | -9        |
| 9 E-LA-EHA-NBA                | 36-18-12-34    | 2540       | 6500       | 2.6 | -21       | -11       |
| 10 E-LA-NBA                   | 42-29-29       | 6380       | 22900      | 3.6 | 9         | -4        |
| 11 E-LA-NBA                   | 44-27-29       | 4440       | 15000      | 3.4 | 9         | 6         |
| 12 E-PHA-NBA                  | 34-22-44       | 4470       | 12900      | 2.9 | -18       | -49       |
| 13 E-C17A-NBA                 | 35-22-43       | 2910       | 8060       | 2.8 | -24       | -50       |
| 14 E-LA-NBA                   | 42-29-29       | 5660       | 23600      | 4.2 | 9         | 6         |
| 15 E-EHA                      | 39-61          | 9780       | 30800      | 3.2 | 9         | -18       |
| 16 E-EHA                      | 38-62          | 8270       | 25200      | 3.0 | 6         | -6        |
| 17 E-EHA                      | 37-62          | 9770       | 28800      | 3.0 | 9         | -16       |
| 18 E-E-EHA-NBA                | 40-31-29       | 10300      | 31900      | 3.1 | 9         | -17       |

## Viscosity and Appearance of the Liquid Ethylene Copolymers

The Kinematic Viscosity at 40° C. (V40) and at 100° C. (V100) were determined according to ASTM D 445. The Viscosity Index (VI) was determined according to ASTM D 2270. The appearance of the liquid ethylene copolymers was determined visually.

The results demonstrated that the ethylene copolymers have a desired high kinematic viscosity, as well as a desired high viscosity index.

TABLE 3

| Viscosity data |              |                |                          |                           |     |
|----------------|--------------|----------------|--------------------------|---------------------------|-----|
| Ex.            | Monomers     | Amounts [wt %] | V40 [mm <sup>2</sup> /s] | V100 [mm <sup>2</sup> /s] | VI  |
| 1              | E-MA         | 34-66          | 17038                    | 372                       | 129 |
| 2              | E-EA         | 32-68          | 3925                     | 185                       | 150 |
| 3              | E-NBA        | 33-67          | 1622                     | 126                       | 177 |
| 4              | E-EHA        | 34-66          | 738                      | 63                        | 154 |
| 5              | E-PHA        | 35-65          | 544                      | 50                        | 150 |
| 6              | E-LA         | 36-60          | 1517                     | 147                       | 209 |
| 7              | E-EHA-NBA    | 32-35-33       | 2202                     | 162                       | 184 |
| 8              | E-LA-NBA     | 35-32-33       | 1536                     | 138                       | 197 |
| 9              | E-LA-EHA-NBA | 36-18-12-34    | 1545                     | 132                       | 183 |
| 12             | E-PHA-NBA    | 34-22-44       | 7701                     | 493                       | 233 |
| 13             | E-C17A-NBA   | 35-22-43       | 2746                     | 195                       | 191 |
| 15             | E-EHA        | 39-61          | —                        | 2943                      | —   |
| 16             | E-EHA        | 38-62          | —                        | 1532                      | —   |
| 17             | E-EHA        | 37-62          | —                        | 2503                      | —   |
| 18             | E-EHA-NBA    | 40-31-29       | —                        | 3725                      | —   |

## Miscibility with Polyalphaolefins

The liquid ethylene copolymers were mixed with polyalphaolefine having a kinematic viscosity at 100° C. of about 6 cSt in a weight ratio of 50:50 at room temperature and mixed at room temperature by rolling for 12 hours. The mixtures' appearance was observed after homogenization and again after 24 hours. The copolymer is deemed compatible with the polyalphaolefine when no phase separation was observed after 24 hours.

The results demonstrated that several of the ethylene copolymers a miscible with very unpolar low viscosity polyalphaolefines (typically based on poly(1-decen)).

TABLE 4

| Miscibility with PAO-6 (50:50 vol %) |              |                |          |
|--------------------------------------|--------------|----------------|----------|
| Ex.                                  | Monomers     | Amounts [wt %] | Miscible |
| 1                                    | E-MA         | 34-66          | No       |
| 2                                    | E-EA         | 32-68          | No       |
| 3                                    | E-NBA        | 33-67          | No       |
| 4                                    | E-EHA        | 34-66          | No       |
| 5                                    | E-PHA        | 35-65          | Yes      |
| 6                                    | E-LA         | 36-60          | Yes      |
| 7                                    | E-EHA-NBA    | 32-35-33       | Yes      |
| 8                                    | E-LA-NBA     | 35-32-33       | Yes      |
| 9                                    | E-LA-EHA-NBA | 36-18-12-34    | Yes      |
| 12                                   | E-PHA-NBA    | 34-22-44       | Yes      |
| 13                                   | E-C17A-NBA   | 35-22-43       | Yes      |

## Hydraulic Oil

The liquid ethylene copolymers can be used in typical hydraulic oils as demonstrated by the following compositions in Table 5. The Lubricants A to D are formulated with commercially available base oils and additives like typical hydraulic oils.

Nexbase® 3043: API Group III base oil, KV40 20 mm<sup>2</sup>/s, KV100 4.3 mm<sup>2</sup>/s, pour point -18° C., commercially available from Neste N.V., Belgium.

Nexbase® 3060: API Group III base oil, KV40 32 mm<sup>2</sup>/s, KV100 6 mm<sup>2</sup>/s, pour point -15° C., commercially available from Neste N.V., Belgium.

- Irgaflo® 942 P: Pour point depressant for lubricants, commercially available from BASF Corp, USA.
- Irgalube® 8080: Ashless anti-wear hydraulic fluid package, commercially available from BASF Corp, USA.
- Additin® RC 9200 N: Zinc containing hydraulic fluid package for antiwear corrosion protection and antioxidant, commercially available from Lanxess, Germany.

TABLE 5

|                            | Hydraulic oil compositions [wt %] |         |         |         |
|----------------------------|-----------------------------------|---------|---------|---------|
|                            | A                                 | B       | C       | D       |
| Nexbase ® 3043             | 20                                | 20      | 15      | 15      |
| Nexbase ® 3060             | 74.9                              | 74.5    | 80.2    | 79.7    |
| Copolymer from Ex. 10      | 4.0                               | 4.0     | —       | —       |
| Copolymer from Ex. 14      | —                                 | —       | 3.7     | 3.8     |
| Irgaflo ® 942 P            | 0.7                               | 0.7     | 0.7     | 0.7     |
| Irgalube ® 8080            | 0.4                               | —       | 0.4     | —       |
| Additin ® RC 9200 N        | —                                 | 0.8     | —       | 0.8     |
| KV40 [mm <sup>2</sup> /s]  | 46.5                              | 46.7    | 45.8    | 47.2    |
| KV100 [mm <sup>2</sup> /s] | 8.5                               | 8.6     | 8.3     | 8.6     |
| Viscosity Index VI         | 160                               | 163     | 157     | 162     |
| Pour point                 | -36° C.                           | -36° C. | -36° C. | -36° C. |
| KRL [%]                    | 5.5                               | 5.5     | —       | —       |

|                            | E    | F    | G    | H    |
|----------------------------|------|------|------|------|
| Nexbase ® 3043             | 25   | 25   | 25   | 25   |
| Nexbase ® 3060             | 69.5 | 69.3 | 68.5 | 69.5 |
| Copolymer from Ex. 15      | 4.0  | —    | —    | —    |
| Copolymer from Ex. 16      | —    | 4.3  | —    | —    |
| Copolymer from Ex. 17      | —    | —    | 4.0  | —    |
| Copolymer from Ex. 18      | —    | —    | —    | 4.0  |
| Irgaflo ® 942 P            | 0.7  | 0.7  | 0.7  | 0.7  |
| Additin ® RC 9200 N        | 0.8  | 0.8  | 0.8  | 0.8  |
| KV40 [mm <sup>2</sup> /s]  | 46.9 | 45.1 | 46.3 | 46.3 |
| KV100 [mm <sup>2</sup> /s] | 8.5  | 8.2  | 8.3  | 8.5  |
| Viscosity Index VI         | 160  | 159  | 157  | 163  |
| Pour point                 | -39  | -36  | -39  | -39  |
| KRL [%]                    | 5.0  | 5.2  | 4.7  | 5.1  |

The data showed, that the hydraulic oils of the compositions A to H have a high viscosity index; have a low pour point; and have a low shear loss, calculated by the KV100 before and after the test according to CEC L-45-99 (20 h) (termed "KRL").

#### Industrial Oil

The liquid ethylene copolymers were used in typical industrial oils, especially gear oil, as demonstrated by the following compositions in Table 6. The Lubricants A to E are formulated with commercially available base oils and additives like typical industrial oils.

The data showed that the industrial oils have an advantageous combination of high viscosity index, low pour point, low shear loss, and good oxidation stability.

PAO 6: a commercially available polyalpholefine having a kinematic viscosity at 100° C. of about 6 cSt.

Group III oil: a commercially available group III base oil with KV100 of 6 cSt.

Ester base stock: Synative® ES DPHA from BASF SE.

Additive Package 1: mixture of commercially available anti-wear additive, metal deactivator, antioxidants, corrosion inhibitor and defoamer.

Ox-Stab.: The oxidation stability was tested according to ASTM D2893 at 121° C., where a sample is subjected to

a temperature of 121° C. for 312 h in the presence of dry air, and then the oil is tested for increase in kinematic viscosity. Table 6 shows the increase in kinematic viscosity in percent.

TABLE 6

|    | Industrial oil compositions [wt %] |         |         |         |         |         |
|----|------------------------------------|---------|---------|---------|---------|---------|
|    | A                                  | B       | C       | D       | E       |         |
| 10 | Copolymer from Ex. 7               |         |         | 53.0    | 53.0    | 56.4    |
|    | Copolymer from Ex. 8               | 55.9    |         |         |         |         |
|    | Copolymer from Ex. 9               |         | 56.9    |         |         |         |
| 15 | PAO 6                              | 40.5    | 39.5    | 43.4    |         | 30.4    |
|    | Group III Oil                      |         |         |         | 43.4    |         |
|    | Ester base stock                   |         |         |         |         | 9.6     |
| 20 | Additive Package 1                 | 3.6     | 3.6     | 3.6     | 3.6     | 3.6     |
|    | KV40 [mm <sup>2</sup> /s]          | 343     | 336     | 305     | 314     | 326     |
|    | KV100 [mm <sup>2</sup> /s]         | 41      | 39      | 35      | 36      | 38      |
|    | Viscosity Index VI                 | 174 w   | 168     | 161     | 159     | 167     |
|    | Pour point                         | -21° C. | -30° C. | -33° C. | -27° C. | -39° C. |
|    | Ox-Stab.                           | 4%      | 5%      | 6%      | 5%      | 6%      |
|    | KRL [%]                            | 8.2     | 3.6     | 2.8     | 3.4     | 3.7     |

The invention claimed is:

1. A lubricant comprising a liquid ethylene copolymer which comprises in polymerized form 20 to 60 wt % of ethylene; and at least 20 wt % of an acrylate, which is selected from  $C_1$ - $C_{22}$  alkyl (meth)acrylate, and wherein the ethylene copolymer is free of further monomers beside the ethylene and the acrylate wherein the acrylate is free of a hydroxyalkyl (meth)acrylate.
2. The lubricant according to claim 1 where the ethylene copolymer has a pour point below 25° C.
3. The lubricant according to claim 1 where the ethylene copolymer has a cloud point of below 25° C.
4. The lubricant according to claim 1 where the ethylene copolymer is miscible with a polyalpholefine having a kinematic viscosity at 100° C. of about 6 cSt.
5. The lubricant according to claim 1 where the ethylene copolymer comprises in polymerized form 25 to 55 wt % of the ethylene.
6. The lubricant according to claim 1 where the ethylene copolymer comprises in polymerized form at least 40 wt % of the acrylate.
7. The lubricant according to claim 1 where the acrylate comprises a polar acrylate selected from  $C_1$ - $C_5$  alkyl (meth)acrylate, and an unpolar acrylate selected from  $C_6$ - $C_{22}$  alkyl (meth)acrylate.
8. The lubricant according to claim 1 where the ethylene copolymer has a number-average molecular weight Mn up to 25000 g/mol.
9. The lubricant according to claim 1 further comprising a base oil selected from mineral oils, polyalpholefins, polymerized and interpolymerized olefins, alkyl naphthalenes, alkylene oxide polymers, silicone oils, phosphate ester and carboxylic acid ester; and/or a lubricant additive.
10. The lubricant according to claim 1 where the ethylene copolymer comprises less than 2 mol % of the vinylester of the formula (I) in polymerized form

27



(I)

where R<sup>c</sup>, R<sup>d</sup>, and R<sup>e</sup> are each independently H or C<sub>1</sub>-C<sub>4</sub>-alkyl, and R<sup>f</sup> is C<sub>1</sub>-C<sub>20</sub> alkyl.

11. A liquid ethylene copolymer as defined in claim 1.

12. A method for reducing friction between moving surfaces comprising the step of contacting the surfaces with the lubricant as defined in claim 1 or with the ethylene copolymer as defined in claim 11.

13. A lubricant comprising a liquid ethylene copolymer which comprises in polymerized form

25 to 55 wt % of ethylene,

at least 20 wt % of the polar acrylate, and

at least 15 wt % of the unpolar acrylate,

comprising

a polar acrylate selected from Ci-05 alkyl (meth)acrylate, and

an unpolar acrylate selected from C6-C22 alkyl (meth)acrylate, and

wherein the ethylene copolymer is free of a hydroxyalkyl (meth)acrylate and comprises in polymerized form.

10

15

20

25

30

35

40

45

50

28

14. The lubricant according to claim 13 where the polar acrylate is selected from C<sub>3</sub>-C<sub>4</sub> alkyl acrylate, and

the unpolar acrylate selected from C<sub>8</sub>-C<sub>22</sub> alkyl acrylate.

15. A lubricant comprising a liquid ethylene copolymer which comprises in polymerized form

20 to 60 wt% of ethylene; and

at least 20 wt% of an acrylate, wherein the acrylate comprises

a polar acrylate selected from Ci-05 alkyl (meth)acrylate, and

an unpolar acrylate selected from C6-C22 alkyl (meth)acrylate

wherein the weight ratio of the unpolar acrylate to the polar acrylate is from 20:80 to 65:35, and

wherein the ethylene copolymer is free of a hydroxyalkyl (meth)acrylate.

16. The lubricant according to claim 15, where the polar acrylate is selected from C3-C4 alkyl acrylate, and

the unpolar acrylate selected from C8-C22 alkyl acrylate.

17. A liquid ethylene copolymer as defined in claim 13.

18. A liquid ethylene copolymer as defined in claim 15.

\* \* \* \* \*